

## UNITED STATES PATENT OFFICE.

CHARLES S. HOLLANDER, OF PHILADELPHIA, PENNSYLVANIA, ASSIGNOR TO ROHM  
& HAAS COMPANY, A CORPORATION OF DELAWARE.

## USE OF SULPHOXYLATES FOR STRIPPING DYES.

No Drawing.

Application filed February 5, 1927. Serial No. 166,272.

The use of sodium sulphoxylate formaldehyde has been suggested as a desirable agent for stripping dyes from animal and vegetable fibres, due to its relatively low 5 cost, its solubility in water and the fact that it need not be used in an alkaline solution (as in the case of sodium hydrosulphite for example) which would have an injurious effect on animal fibres. However, experience 10 has shown that this substance has a tendency to break down too rapidly and deposit sulphur on the goods, which seriously interferes with subsequent dyeing operations. 15 The present invention relates to a method whereby sodium sulphoxylate formaldehyde can be used advantageously, and is based upon my discovery that if the sodium salt is combined with a water-soluble salt of zinc, 20 the sodium salt will be stabilized and give very efficient results. Zinc salts that may be used for this purpose include zinc sulphate, zinc chloride, zinc acetate or other salts of a similar nature. Inasmuch as it is desir- 25 able to add more or less acid to the stripping bath, some or all of the zinc may be added in a form which will combine with such acid to form a soluble zinc salt. For example, zinc oxide and sulphuric or acetic 30 acid may be added instead of zinc sulphate or zinc acetate. However, in this case, as in the other, the bath will comprise a solution of sodium formaldehyde sulphoxylate mixed with a soluble zinc salt. 35 In this case, as in my earlier Patent No. 1,594,670, dated August 3, 1926, an equilibrium is established, but whereas in the former case the equilibrium involved some insoluble ingredients, in the present case all 40 of the essential ingredients are soluble, for zinc hydroxide is not necessarily present as before and the soluble normal zinc sulphoxylate formaldehyde is present instead of the substantially insoluble basic compound, as 45 shown by the following formula:



While the amount of zinc used may be varied within substantial limits, I find that 50 efficient results can be obtained by using about half as much of the zinc salt as of the sulphoxylate; for example, 70% of sodium formaldehyde sulphoxylate and 30% of anhydrous zinc sulphate will give good results.

These figures are not intended as a limitation, but are only given to show that substantial quantities of the zinc salt should be used.

The following is an example of my process:

Rags were first boiled with enough water to cover them, to which had been added about 5% of ammonia. This operation removed the dirt and grease and also extracted a considerable amount of dye. The goods 65 were then thoroughly rinsed and heated to between 120 and 140° F. with enough water thoroughly to cover them. Between 1/2 and 1% of acid (such as sulphuric, acetic, or formic) was added and thoroughly mixed in 70 and then 5% of a mixture of 70% sodium formaldehyde sulphoxylate with 30% of anhydrous zinc sulphate was introduced, and the water was heated until a temperature of between 190 and 200° F. was reached. After 75 the goods had been heated for some time in this bath the dyes were found to be destroyed; the liquor was discarded and the goods thoroughly rinsed.

For the purposes of convenience, the sodium formaldehyde sulphoxylate and the zinc salt may be prepared in dry powdered form and mixed together in the proper proportions and stored or sold mixed together. They are then immediately available for use 85 in preparing an efficient stripping bath.

What I claim is:

1. The process of stripping dyes from fibres which comprises the step of soaking such fibres in a heated bath comprising dissolved substances in equilibrium, such substances comprising sodium sulphoxylate formaldehyde and a soluble zinc salt on the one hand and soluble zinc sulphoxylate formaldehyde and a soluble sodium salt on the other hand.

2. The method of preparing a bath for stripping dyes from fibres which comprises the steps of dissolving together sodium sulphoxylate formaldehyde and a soluble zinc salt whereby an equilibrium of soluble ingredients is obtained comprising sodium sulphoxylate formaldehyde and zinc sulphoxylate formaldehyde.

3. A composition of matter adapted for 105 use in the production of a bath for stripping dyes comprising sodium sulphoxylate formaldehyde and a substantial amount of a

soluble zinc salt, mixed together in powdered form, and adapted when dissolved in water to form a bath comprising dissolved substances in equilibrium, such substances comprising sodium sulphoxylate formaldehyde and a soluble zinc salt on the one hand and soluble zinc sulphoxylate formaldehyde

and a soluble sodium salt on the other hand.

4. A composition as specified in claim 3 in which the amount of soluble zinc salt is about half of the amount of sodium formaldehyde sulphoxylate. 10

CHARLES S. HOLLANDER.